

## UNITED STATES PATENT OFFICE

2,426,674

## NONSTRETCH GARMENT

Camille Dreyfus, New York, N. Y.

No Drawing. Application January 3, 1945,  
Serial No. 571,211

2 Claims. (Cl. 2—243)

1

This invention relates to wearing apparel of high dimensional stability, and relates more particularly to non-stretching, non-shrinking wearing apparel formed of fabrics made of or containing regenerated cellulose yarns and threads having a basis of a stretched and saponified organic acid ester of cellulose.

An object of this invention is the provision of improved garments which possess high dimensional stability.

Another object of this invention is the production of outer garments and under garments which resist any change in dimensions as by shrinking or stretching even after repeated laundering or other cleansing operations.

A further object of this invention is the provision of dimensionally stable garments wherein the seams and other sewn or stitched portions thereof will retain a neat and unwrinkled appearance.

Other objects of this invention will appear from the following detailed description.

It has been long observed that garments and other forms of apparel prepared from fabrics of various materials, for example, cotton, undergo some degree of shrinkage in the body of the garment and in the seams when subjected to laundering or like cleansing operations. In order to overcome the obvious disadvantages of such shrinkage, the garments must either be cut and sewn in such a manner that after laundering and its usual shrinking effect, they will be the size ultimately desired, or else the fabric employed must be so treated prior to cutting that any subsequent shrinkage will be kept at a minimum. Normally, the latter expedient is employed. Cutting garments oversize to allow for shrinkage is quite impractical. The degree of shrinkage in the direction of the warp may vary considerably from that in the direction of the weft, and these directional variations in shrinkage may differ markedly in fabrics of different construction. While preshrunk fabrics appear to offer the most practical means of eliminating the disadvantages of garment shrinkage, such preliminary treatment of the fabrics, though adding to the cost, offers no guarantee that they will retain their original dimensions permanently. There is usually some residual shrinkage which remains. This residual shrinkage, coupled with the fact that the threads employed for sewing also tend to shrink to a substantial degree ultimately produces at least along the seams of the garments an uneven, wrinkled and buckled condition which is quite unsatisfactory.

2

I have now discovered that the aforementioned and other disadvantages may be entirely eliminated if the fabrics of which said garments are formed and the threads employed for sewing the fabrics of which said garments are formed comprise dimensionally stable regenerated cellulose textile materials having a basis of stretched and saponified organic acid ester of cellulose yarns. These regenerated cellulose materials which are

10 prepared by stretching and saponifying processes, are remarkable for their dimensional stability, neither shrinking nor stretching in service notwithstanding severe and repeated laundering, wide variations in temperature conditions, or as 15 a result of the continuous or intermittent application of a substantial pull or tension on the garments during service. Furthermore, since the undesirable effects of shrinking are eliminated, the seams of my novel garments retain their original smooth and even appearance permanently.

The filaments from which the stretched and saponified regenerated cellulose threads and fabrics are prepared may be formed by extruding a solution of cellulose acetate or other organic 25 ester of cellulose in a suitable volatile solvent through an orifice into an evaporative medium as in the dry method of spinning, or into a coagulating medium as in the wet method of spinning. A plurality of filaments may be extruded through 30 several orifices and associated to form a yarn or thread. The yarns or threads obtained may be stretched simultaneously with their formation, or subsequent to their formation after first being softened by means of a suitable softening medium 35 such as, for example, solvent vapors, steam, hot water or even dry heat. The softened yarns may be stretched 300, 500, 1000 or even 2000% or more of their original length during the stretching operation. Stretching greatly increases the 40 tenacity of the yarns while lowering the elongation, and this increase in tenacity is retained and frequently increased substantially when the stretched organic ester of cellulose yarns are saponified so that a regenerated cellulose yarn is 45 obtained.

The saponification of the organic ester of cellulose yarns may be carried out employing any suitable basic agent. Inorganic saponifying agents such as aqueous solutions of sodium hydroxide, potassium hydroxide, sodium silicate, sodium carbonate or ammonium hydroxide are satisfactory. Organic saponifying agents, for example, ethyl amine, methyl amine or other organic bases may also be employed. Saponification may 55 be effected at temperatures of 20 to 100° C. When

employing aqueous solutions of sodium hydroxide, for example, as the saponifying agent, said solutions may be of a concentration of 0.1 to 5% by weight and saponification may be effected at temperatures of 30 to 90° C. in 30 to 180 minutes. Usually, when employing aqueous saponifying solutions comprising sodium hydroxide, a salt such as sodium chloride or sodium acetate is advantageously added to the saponifying baths.

Other organic esters of cellulose which may be stretched and saponified to yield regenerated cellulose yarns of high dimensional stability, are, for example, cellulose propionate, cellulose butyrate, and mixed esters such as cellulose acetate-propionate, and cellulose acetate-butyrate.

The regenerated cellulose yarns which are obtained on saponification may then be woven into fabrics of any desired construction. A suitable number of the regenerated cellulose filaments may be plied or associated together in any desired fashion and twisted to form sewing threads. Normally the regenerated cellulose yarns obtained have an elongation of not more than 0.3% over a variation in relative humidity of 10 to 100%, which degree of elongation is about 85% less than any comparable textile material such as, for example, silk. Furthermore, as stated, these regenerated cellulose yarns do not shrink as a result of laundering nor do they stretch appreciably under tension.

The garments for which the regenerated cellulose textile materials are especially suitable are, for example, shirts wherein the permanent fit of the collar portion and permanent flatness of the seams are exceedingly important, undergarments such as girdles, brassières and corsets where any shrinkage as a result of washing, or stretching as a result of use, impairs the fit and utility of the garment, orthopedic garments and

devices where permanent dimensional stability of the fabric portion is exceedingly important to effect the desired support, and like garments in which the absolute permanence of the original dimensions measures the value and serviceability of the garment.

It is to be understood that the foregoing detailed description is given merely by way of illustration and that many variations may be made therein without departing from the spirit of my invention.

Having described my invention, what I desire to secure by Letters Patent is:

1. Garments of high dimensional stability and non-buckling seams resistant to shrinking or stretching as a result of laundering or hard service, comprising fabrics of yarns of regenerated cellulose sewn with regenerated cellulose threads, said regenerated cellulose yarns and threads being prepared by stretching and saponifying yarns having a basis of an organic ester of cellulose.

2. Garments of high dimensional stability and non-buckling seams resistant to shrinking or stretching as a result of laundering or hard service, comprising fabrics of yarns of regenerated cellulose sewn with regenerated cellulose threads, said regenerated cellulose yarns and threads being prepared by stretching and saponifying yarns having a basis of cellulose acetate.

30

CAMILLE DREYFUS.

## REFERENCES CITED

The following references are of record in the file of this patent:

## FOREIGN PATENTS

|         |               |               |
|---------|---------------|---------------|
| Number  | Country       | Date          |
| 542,773 | Great Britain | Jan. 27, 1942 |